

# United States Patent Office

2,828,351

Patented Mar. 25, 1958

1

2,828,351

ANODES

Henry R. Rade, Cleveland, Ohio, assignor to Union Carbide Corporation, a corporation of New York

No Drawing. Application November 17, 1953  
Serial No. 392,745

6 Claims. (Cl. 136—126)

This invention relates to consumable metal anodes for primary galvanic cells, and to an improved method of constructing such anodes.

Beginning with the early Leclanché type cells, anodes for primary galvanic cells have been cast or fabricated from sheet metal. In relatively large cells such as those used for railway signal service, telephone service, or for flashlights, and similar devices of relatively large size anodes of this type are perfectly satisfactory. Recently, however, due to the development of electronic devices of smaller size, such as the personal hearing aid and portable radio transmitters and the like, there has been a demand for the production of primary batteries of small size. The continuing trend is to reduce the size of such batteries even further.

As the size of primary cells has been decreased, difficulties have been encountered with the anode materials used. The smaller the anode, the greater the difficulty. One of the reasons for such difficulties is the lack of surface of anode material which can be attacked by the electrolyte. The small anode of sheet metal tends to become coated with current-stopping reaction products in so short a time as to render the cell commercially undesirable.

To counter-balance the decrease in anode size necessitated by the continued decrease in cell size, many attempts have been made to increase the effective surface area to insure more complete utilization of the anodic material. For example, a sheet metal anode may be embossed or perforated not only to provide more surface area, but also to prevent adherence to the anode of non-conductive reaction products. While such expedients have been effective to a degree, they have not solved the problem.

Another way of effecting a desired extension in anode surface area which has been adopted to some extent commercially, consists in forming the anode of powdered metal; for example, by compressing powdered anodic material into the form of a cylinder. Anodes so formed have a greater effective surface area than a cylinder of the same size cast from molten metal. However, anodes compressed of metal powders in themselves suffer disadvantages. If an anode so formed is compressed with too little pressure, there results a structurally weak element, while on the other hand if too much pressure is used in the formation of such anodes, an appreciable part of the resultant anode will be unattacked by electrolyte, and therefore, will contribute nothing to the cell reaction. Additionally, powdered metal anodes made in this way are porous, and permit internal electrolytic action during cell discharge with the consequent formation of reaction products within the pores of the anode. Since these reaction products occupy considerably more space than the anode metal, internal pressure develops in the anode, which often results in spalling and breaking apart.

It is the principal object of this invention to provide anode material having greater effective surface area than

2

anodes of smaller size fabricated from sheet or cast metal, and yet which is free of the disadvantages of anodes formed of compressed metal powder, another object of the invention is a method of producing such anodes.

5 In accordance with the invention, these objects are achieved by an anode composed of finely divided anode metal bonded into a desired shape by an electrolyte-repellent, electrically non-conductive, flexible, thermoplastic material. This invention also includes a method of bonding with a thermoplastic resin finely divided anode metal by compression under heat and pressure.

The most widely used anode material in primary galvanic cells is zinc, and for the purpose of conciseness, the invention will be described particularly with reference to zinc anodes. However, the invention is equally applicable to the production of anodes formed of any consumable metal, for example, magnesium or aluminum.

Anodes made in accordance with the invention are composed of finely divided anode metal bonded into 20 the desired shape by a relatively small proportion of a thermoplastic binder, the binder forming a continuous plastic matrix throughout the anode, and the anode metal itself forming a continuous phase. Suitable binding materials include polyethylene, polyvinyl chloride, ethyl cellulose, vinyl resins and chlorinated diphenyl resins. Of this group, polyethylene is preferred because of its excellent heat tolerance.

The proportion of binder to anode metal in the anodes of this invention is desirably as small as possible, commensurate with securing reasonable mechanical strength. Ordinarily, the binder should constitute at least about 1% by weight of the anode, and larger quantities may be used, commensurate with the reduction in electrical conductivity of the formed anode encountered as the proportion of binder is increased. For most purposes, the proportion of binder need not exceed 5% of the anode, and generally is well below 5%.

The desity of the anode, of course, is dependent upon the ratio of metal to resin in the mixture.

40 Thus in determining the quantity of thermoplastic binder to be used in making the anodes of the invention, ease of molding is an important consideration, but even more important is the necessity for providing in the anode the maximum possible quantity of active anode metal. As little as 1% by weight of powdered resin may be used to fill the interstices between the particles, and mixtures containing only this small proportion of binder may be molded with relative ease. Whenever greater ease of molding is desired, larger quantities of the resin may be used, but it must be borne in mind that the finished article must have satisfactory electrical conductivity for its intended purpose, and the maximum quantity of binder that can be used is that which causes no undue decrease in the electrical conductivity of the finished anode. Numerically, this upper limit is approximately 12%.

45 In manufacturing the anodes of this invention, powdered anode metal is dry-mixed with powdered binder resin. Although particle size of the metal is not critical, it is convenient to employ powders of such a size that they will pass a 40 mesh (0.417 mm.) screen, while being retained on a 170 mesh (0.088 mm.) screen, and the resin particles should generally be of the same order. The blended mixture is compressed in conventional manner under suitable conditions of elevated temperature and pressure to form any desired shape of anode. Generally, dependent upon the resin selected, the temperature should be at least about 200° F., and the pressure applied, which is in part dependent upon the quality of resin in the mixture, should be at least about 1000 pounds per square inch. Typical examples of suitable mixtures and molding conditions follow.

Cylindrical anodes  $\frac{3}{8}$ " in outside diameter by  $\frac{5}{16}$ " height were prepared from a mixture containing 99% zinc having a particle size such as to pass a 40 mesh (0.417 mm.) screen, and 1% polyethylene and successfully molded at 300° F. and a pressure of 2000 pounds per square inch.

From a mixture composed of 97.5% zinc and 2.5% polyethylene, the zinc having a particle size sufficiently small to pass a 40 mesh (0.417 mm.) screen, cup-shaped anodes having an outside diameter of  $\frac{3}{8}$ ", a length of  $1\frac{5}{8}$ " and a side wall thickness of 0.012" were molded at 350° F. and 3000 pounds per square inch pressure.

Anodes in the form of rods of varying lengths having a diameter of  $\frac{5}{16}$ " were molded at 400° F. and 3500 pounds per square inch pressure, from a blend consisting of 200 grams of powdered zinc and 10 grams of powdered polyethylene, the zinc powder was of a particle size sufficiently small to pass through a 40 mesh (0.417 mm.) screen.

Anodes typical of those just described when subjected to the action of electrolyte, are uniformly corroded in such a way that complete utilization of the anode metal is achieved. Actually, corrosion, upon which of course battery action depends, proceeds so uniformly and so completely that when the anodes are immersed in electrolyte, complete consumption of the anode metal can be attained, leaving behind a coherent matrix of thermoplastic binder, which still retains the shape of the original anode. Furthermore, reaction proceeds from the outside surfaces of the anode progressively as the anode is consumed without any tendency to breakage of the anode by spalling, indicating that electrolytic action within the interior portions of the anode is inhibited.

This inhibition of internal electrolytic action conceivably may be due to a lack of porosity of the anode or to the fact that the binder resin has an electrolyte-repellent property or to both of these phenomena. Whatever the explanation, however, the fact remains that the anodes of the invention are uniformly corroded at the active surfaces thereof, rather than in the interior portion. This characteristic assures uniform service life of batteries employing the anodes, and prevents early failure of such batteries prior to the complete utilization of the anode metal.

As has been indicated above, a relatively large number of thermoplastic resins may be utilized as the binder in forming the anodes of this invention. Of the group above referred to, polyethylene is preferred because its excellent heat tolerance enables anodes made in accordance with this invention, utilizing polyethylene as a binder, to be soldered by standard methods without undergoing structural deformation.

A particular advantage of the invention lies in the fact that anodes of any desired shape may be produced with

ease, thereby freeing the battery maker from the necessity of employing the shapes traditionally used. Further advantages accrue from the fact that pure metal may be employed, and that uniformity of composition may thereby be achieved. Such uniformity eliminates the possibility of the development of local couples in cells or batteries employing the anodes which tend to shorten battery life. Additionally, by reason of the continuity of both matrix and anode metal, substantially complete utilization of the anodic metal may be achieved.

I claim:

1. A primary galvanic cell anode composed of 99% of powdered zinc metal, and 1% of polyethylene powder.

15 2. An easily soldered primary galvanic cell anode comprising 97½% of zinc metal and 2½% of polyethylene powder.

3. A cup-shaped primary galvanic cell anode comprising 99% of powdered zinc metal, and 1% of polyethylene powder.

20 4. A cup-shaped primary galvanic cell anode comprising 97½% of zinc metal, and 2½% of polyethylene powder.

25 5. A molded self-supporting anode for primary galvanic cells, said anode comprising finely divided particles of an anodic metal selected from the group consisting of zinc, aluminum and magnesium, said particles being integrally united by a plastic resin selected from the group consisting of polyethylene, ethyl cellulose and chlorinated diphenyl resins, said resin constituting a substantially continuous matrix and being present throughout said anode in an amount ranging from 1 percent to 12 percent by weight thereof.

30 6. A molded self-supporting anode for primary galvanic cells, said anode comprising finely divided particles of an anodic metal selected from the group consisting of zinc, aluminum and magnesium, said particles being integrally united by a plastic resin selected from the group consisting of polyethylene, ethyl cellulose and chlorinated diphenyl resins, said resin constituting a substantially continuous matrix and being present throughout said anode in an amount ranging from 1 percent to 5 percent by weight thereof, said metal and said resin having a particle size ranging from 0.088 millimeter to 0.417 millimeter.

35 45

#### References Cited in the file of this patent

#### UNITED STATES PATENTS

|    |           |               |               |
|----|-----------|---------------|---------------|
| 50 | 2,623,915 | Moulton       | Dec. 30, 1952 |
|    | 2,677,713 | Weil et al.   | May 4, 1954   |
|    | 2,694,743 | Ruskin et al. | Nov. 16, 1954 |
|    | 2,708,683 | Eisen         | May 17, 1955  |
|    | 2,737,541 | Collidge      | Mar. 6, 1956  |
| 55 | 2,738,375 | Schlotter     | Mar. 13, 1956 |